# EUROPEAN PATENT SPECIFICATION

(11) **EP 0 547 084 B1**
(45) Date of publication and mention of the grant of the patent: **10.08.1994**
(21) Application number: 91915056.5
(22) Date of filing: 03.09.1991
(51) Int. Cl.: G03C 5/42, G03C 11/04

(54) **SILVER IMAGE BLEACHING PROCESS**
SILBERBILDBLEICHVERFAHREN
PROCEDE DE BLANCHIMENT D'IMAGES ARGENTIQUES

(30) Priority: 07.09.1990 GB 9019604
(43) Date of publication of application: 23.06.1993
(73) Proprietor: KODAK LIMITED, Harrow, Middlesex HA1 4TY (GB); EASTMAN KODAK COMPANY (a New Jersey corporation), Rochester, New York 14650 (US)
(72) Inventor: BARNETT, Anthony Malcolm, Harrow, Middlesex, HA1 4TY (GB); HALLBERY, David Alan, Harrow, Middlesex, HA1 4TY (GB)
(74) Representative: Baron, Paul Alexander Clifford
(86) International application number: EP9101659
(87) International publication number: WO9204659

(56) References cited:
- BE-A- 1 002 506
- DE-A- 590 919
- US-A- 2 108 261
- US-A- 2 141 354
- US-A- 2 206 190
- US-A- 3 423 441
- World Patents Index, Week 8040, Derwent Publications Ltd., London, GB; AN 80-70519C & JP,A, 55 109 210

## Description

This invention relates to a method of bleaching silver images and to solutions therefor.

The photographic silver halide image forming process is well known. Sometimes it is desirable to retouch the silver image formed thereby and, specifically, it is sometimes desired to remove parts of the image such as unwanted spots.

It is known, for example from British specification 2 107 889 that a thickened solution containing, for example, iodine and an iodide can achieve the desired result. A problem with this approach is that a brown stain is produced which is unsightly. In addition the compositions of 2 107 889 are only suitable for printing plates which do not have any gelatin layers. It is therefore desirable to be able to delete the silver image without causing any stain and to delete the silver image in a gelatin-containing layer.

The present invention provides a method of removing silver images without causing any stain.

According to the present invention there is provided a method for bleaching a silver image wherein the image is treated with a first solution comprising iodine and an iodide salt and then the iodine stain is removed by treating it with a second solution containing from 10 to 100g ascorbic acid and from 10 to 100g (as potassium sulphite) of sulphite ions per litre.

The image is bleached rapidly and permanently, there is no stain and the solutions have a long life.

The silver image to be treated may be on an imagewise exposed and fully processed photographic film or paper or on a printing plate made by the photographic silver salt diffusion transfer process. Such materials are described in Research Disclosure Item 308119, December 1989 published by Kenneth Mason Publications, Emsworth, Hants, United Kingdom.

In a preferred embodiment of the present invention the solutions are applied to the silver image using "felt tipped" pens, preferably ones with a fine tip to ensure accurate application.

The first solution, used to delete the silver image preferably contains a mixture of water and butyrolactone. The ratio of aqueous to organic solvent is optimised to provide sufficient water for rapid penetration of the solute into the gelatin layer on the image-bearing material, together with sufficient butyrolactone to obtain high complexing power for silver iodide so that the image is removed in a conveniently quick time. The first may also contain other solvents used alone or in combination including alcohols eg ethyl or butyl alcohol.

The iodide may be provided by an ammonium or alkali metal iodide, eg sodium or potassium iodide.

The first solution preferably contains from 2 to 50g, especially from 20g to 45g, of iodine and from 50g to 250 g, especially from 150g to 200g, of iodide ions per litre. The solvent preferably comprises from 10 to 60% by weight of water, the exact figures being dependent on the considerations outlined above. Preferably the first solution also contains a wetting agent and an acid.

The second solution preferably contains from 40 to 80g ascorbic acid and from 30 to 70g of potassium sulphite per litre. The solution is preferably aqueous.

The invention further provides a deletion fluid kit comprising the first and second solutions as defined above. Preferably the solutions are each contained in a felt tip pen.

The following Example is included for a better understanding of the invention. The words KODAK and PMT are trademarks.

### EXAMPLE

The following solutions were made up:

### SOLUTION A

### SOLUTION B

Each solution was filled into a felt tip pen.

Images were produced using Kodak PMT3 KNP negative paper, exposed on a Kodak Imagemaker Camera and processed in a Kodak 43DT Imagemate Processor onto a variety of Kodak PMT receivers. Images were deleted successfully from the following receivers in an average time of 20 seconds.
- PMT 3: KRPM Matt receiver paper
- PMT 3: KRPT Thin receiver paper
- PMT 3: KRPTA Adhesive thin receiver paper
- PMT 3: KRPG Glossy receiver paper
- PMT 3: KRF Receiver film
- PMT 3: KRFT Thin receiver film
- PMT II: Metal litho plates

Other materials tried were Kodak PMT II Paper Litho plates and Kodak Pagiset Phototypesetting paper. Images could be successfully deleted from both, but the deletion time was greater than 1 minute.

## Claims

1. A method for bleaching a silver image wherein the image is treated with a first solution comprising iodine and an iodide salt and then the iodine stain is removed by treating it with a second solution containing from 10 to 100g ascorbic acid and from 10 to 100g (as potassium sulphite) of sulphite ions per litre.

2. A method as claimed in claim 1 in which the silver image to be treated is located on an imagewise exposed and fully processed photographic film or paper or on a printing plate made by the photographic silver salt diffusion transfer process.

3. A method as claimed in Claim 1 or 2 in which the solutions are applied to the silver image using felt tipped pens.

4. A method as claimed in any of claims 1 - 3 in which the first solution contains from 2 to 50g, preferably from 20g to 45g, of iodine per litre.

5. A method as claimed in any of claims 1 - 4 in which the first solution contains from 50 to 250 g, preferably from 150g to 200g, of potassium iodide per litre.

6. A method as claimed in any of claims 1 - 5 in which the solvent of the first solution comprises from 10 to 60% by weight of water.

7. A method as claimed in any of claims 1 - 6 in which the second solution comprises an aqueous solution containing from 40 to 80g ascorbic acid and from 30 to 70g of potassium sulphite per litre.

8. A deletion fluid kit comprising the first and second solutions as defined in any of claims 1 - 2 and 4 - 7.

9. A deletion fluid kit as claimed in claim 8 in which the solutions are each contained in a felt tip pen.

## Patentansprüche

1. Verfahren zum Ausbleichen eines Silberbildes, bei dem das Bild mit einer ersten Lösung behandelt wird, die Iod und ein Iodidsalz enthält, worauf die Iodverfärbung entfernt wird durch Behandlung mit einer zweiten Lösung, die 10 bis 100 g Ascorbinsäure und 10 bis 100 g Sulfitionen (als Kaliumsulfit) pro Liter enthält.

2. Verfahren nach Anspruch 1, bei dem sich das zu behandelnde Silberbild auf einem bildweise exponierten und voll entwickelten photographischen Film oder Papier oder einer Druckplatte, hergestellt nach dem photographischen Silbersalzdiffusionsübertragungsverfahren, befindet.

3. Verfahren nach Anspruch 1 oder 2, bei dem die Lösungen auf das Silberbild mittels Filzstiften aufgebracht werden.

4. Verfahren nach einem der Ansprüche 1 bis 3, bei dem die erste Lösung 2 bis 50 g, vorzugsweise 20 g bis 45 g Iod pro Liter enthält.

5. Verfahren nach einem der Ansprüche 1 bis 4, bei dem die erste Lösung 50 bis 250 g, vorzugsweise 150 g bis 200 g, Kaliumiodid pro Liter enthält.

6. Verfahren nach einem der Ansprüche 1 bis 5, bei dem das Lösungsmittel der ersten Lösung 10 bis 60 Gew.-% Wasser enthält.

7. Verfahren nach einem der Ansprüche 1 bis 6, bei dem die zweite Lösung eine wäßrige Lösung umfaßt, die 40 bis 80 g Ascorbinsäure und 30 bis 70 g Kaliumsulfit pro Liter enthält.

8. Flüssiger Lösch-Kit mit der ersten und der zweiten Lösung gemäß einem der Ansprüche 1 bis 2 und 4 bis 7.

9. Lösch-Kit nach Anspruch 8, in dem die Lösungen jeweils in einem Filzstift enthalten sind.

## Revendications

1. Procédé pour blanchir une image argentique dans lequel l'image est traitée avec une première solution comprenant de l'iode et un sel iodure puis la coloration due à l'iode est éliminée par traitement avec une seconde solution contenant de 10 à 100 g/l d'acide ascorbique et de 10 à 100 g/l d'ions sulfite sous forme de sulfite de potassium.

2. Procédé selon la revendication 1 dans lequel l'image argentique à traiter se trouve sur un film ou papier photographique exposés conformément à l'image et traités complètement ou sur une plaque d'impression obtenue par un procédé photographique de transfert par diffusion du sel d'argent.

3. Procédé selon la revendication 1 ou 2 dans lequel les solutions sont appliquées sur l'image argentique en utilisant des crayons feutres.

4. Procédé selon les revendications 1 à 3 dans lequel la première solution contient 2 à 50 g/l et de préférence 20 à 45 g/l d'iode.

5. Procédé selon l'une quelconque des revendications 1 à 4 dans lequel la première solution contient 50 à 250 g/l et de préférence 150 à 200 g/l d'iodure de potassium.

6. Procédé selon l'une quelconque des revendications 1 à 5 dans lequel le solvant de la première solution comprend 10 à 60 % d'eau en poids.

7. Procédé selon l'une quelconque des revendications 1 à 6 dans lequel la seconde solution comprend une solution aqueuse contenant 40 à 80 g d'acide ascorbique et 30 à 70 g/l de sulfite de potassium.

8. Ensemble de fluides pour l'effacement d'une image argentique comprenant une première et une seconde solutions telles que définies dans l'une quelconque des revendications 1-2 et 4-7.

9. Ensemble de fluides pour l'effacement d'une image argentique selon la revendication 8 dans lequel les solutions sont chacune contenues dans un crayon feutre.
